# EUROPEAN PATENT SPECIFICATION

(11) **EP 0 629 686 B1**
(45) Date of publication and mention of the grant of the patent: **22.07.1998**
(21) Application number: 94900321.4
(22) Date of filing: 20.10.1993
(51) Int. Cl.: C10L 1/06, C10L 1/30

(54) **FUEL COMPOUND FOR INTERNAL COMBUSTION ENGINES**
BRENNSTOFFVERBINDUNG FÜR BRENNKRAFTMASCHINEN
COMPOSE DE CARBURANT POUR MOTEURS A COMBUSTION INTERNE

(30) Priority: 22.10.1992 RU 9201874
(43) Date of publication of application: 21.12.1994
(73) Proprietor: AKTSIONERNOE OBSCHESTVO" ACHINSKY NEFTEPERERABATYVAJUSCHY ZAVOD", Achinski, 662114 (RU)
(72) Inventor: DEMYANENKO, Egor Alexandrovich, Achinsk, 662100 (RU); BIRJUKOV, Felix Ivanovich, Achinsk, 662100 (RU); KARIBOV, Alisker Karibovich, Achinks, 662100 (RU); SACHIVKO, Alexei Vladislavovich, Krasnoyarsk, 660028 (RU); TEMEROV, Sergei Anatolievich, Krasonyarsk, 660059 (RU); TVERDOKHLEBOV, Vladimir Pavlovich, Krasnoyarsk, 660060 (RU); EMELYANOV, Vyacheslav Evgenievich, Moscow, 111123 (RU); RADCHENKO, Evgeny Dmitrievich, Moscow, 121165 (RU)
(74) Representative: Woods, Geoffrey Corlett
(86) International application number: RU9300239
(87) International publication number: WO9409091

(56) References cited:
- DE-B- 1 289 357
- FR-A- 1 140 411
- US-A- 2 810 737
- US-A- 3 377 248
- US-A- 4 336 033
- US-A- 4 389 220
- DATABASE WPI Week 9432, Derwent Publications Ltd., London, GB; AN 94-261972 & SU-C-2 006 497 (DEMYANENKO ET AL.) 30 January 1994

## Description

The present invention relates to lead compound free high-octane fuel compositions for internal combustion engines with spark ignition, prepared by using hydrocarbon fuels and anti-knock additive.

There are known fuel compositions based on hydrocarbon fuels containing ferrocene derivatives as anti-knock additive such as m-nitrocinnamoyl ferrocene and o-chlorocinnamoyl ferrocene ( Toma,P.Ele ko, V.Vesely and M.Sali ova: Derivaty ferocenu ako prisady do benzinov. Acta Facultatis rerum naturalium universitatis comenianae-formatio et protectio naturae 1981 No. 7, 187-192 (Ref Journal CHEMISTRY, 12, II 224 (1982))

In addition, US-A-2810737 describes alpha-hydroxyalkyl ferrocene derivatives and their use as anti-knock agents in spark ignition fuels.

A considerable obstacle for using ferrocene and its derivatives as an anti-knock additive to the engine fuels is that in the combustion chamber, more specifically on sparking plugs some deposits of iron oxides are formed, causing some failures in the operation of an engine (E.G. Perevalova, M.D. Reshetova, K.I. Granberg, "Methods of Elementorganic Chemistry", Moscow, Publishing House NAUKA, 1983, p. 439 (Russian edition)).

In addition said m-nitrocinnamoylferrocene and o-chlorocinnamoylferocene are produced from ferrocene in a number of stages with a low yield and all characterized with a low solubility rate in the fuel composition.

It is an object of the present invention to create a high octane fuel composition for internal combustion engines eliminating said drawbacks.

Accordingly, the present invention provides a hydrocarbon based fuel composition suitable for spark ignition internal combustion engines, which comprises 0.001% - 0.02% by weight of

Typically the hydrocarbon composition comprises:

| | |
|---|---|
| aromatic hydrocarbone | 54 to 56 percent by weight. |
| normal alkanes | 12 to 13 percent by weight. |
| isoalkanes | 29 to 31 percent by weight. |
| naphtheness | 1 to 2 percent by weight. |

Such a composition has fractions as follows:

| | | |
|---|---|---|
| initial boiling point: | | 60 grad.C |
| distillation | fraction of 10 percent; | 83 grad.C |
| distillation | fraction of 50 percent: | 114 grad.C |
| distillation | fraction of 90 percent: | 156 grad.C |
| distillation | fraction of 96 percent: | 190 grad.C |

density p20/4 being 0.7687 g/cm³ and motor octane number being 80.

The present invention further provides the use of as an anti-knock additive suitable for fuels.

### Examples and Comparative Examples

The fuel composition octane number was determined on the plant UIT-85 by a motor method according to OMEA Standard 2243-80. The plug operation-to-failure time was determined on the single cylinder compartment of the engine ZIL-130 at alternative modes covering a wide spectrum of changed parameters such as temperature of cooling liquid, load, ingredients of mixture and lead angle of ignition. The test was carried out by some five-hour cycles.

Iron oxide on the sparking plug A11 with an initial gap being 0.64 mm was appreciated by parameters as follows: change of sparking gap, change of the sparking plug weight, iron oxide deposit surface nature on the sparking plug electrodes. The sparking gap was measured by using the projector type SVET with magnification X100 and the iron oxide deposit surface nature was estimated by means of an optical microscope type MIN-8 with magnification X50.

The fuel composition was tested by using, as anti-knock additive, a ferrocene derivative corresponding to the prior art (Nos 1. to 6 in the following Table) and a ferrocene derivative in different amounts according to the present invention (Nos. 7 to 10 in the following Table).

**TABLE**

| No. | Dosage of Additive | Motor Octane | Time Hour | Increased Weight | Spark gap | Deposit on plug |
|---|---|---|---|---|---|---|
| 1 | 2 | 3 | 4 | 5 | 6 | 7 |
| 1 | m-nitro- | 81.9 | - | - | 640 | Homogeneous |
| | cinnamoyl | (1.9) | 5 | 4 | 635 | dense |
| | ferrocene | | 10 | 8 | 630 | varnished |
| | 0.0296 | | 15 | 13 | 625 | deposit |
| | (0.00459) | | 20 | 16 | 605 | |
| | | | 25 | 24 | 595 | |
| | | | 30 | 33 | 580 | |
| | | | 35 | 40 | 560 | |
| | | | 40 | 50 | 525 | |
| | | | 45 | stop | | |
| 2 | m-nitro- | 81.6 | - | - | 640 | Homogeneous |
| | cinnamoyl | (0.2) | 5 | 0 | 640 | dense |
| | ferrocene | | 10 | 2 | 635 | varnished |
| | 0.0148 | | 15 | 3 | 635 | deposit |
| | (0.00229) | | 20 | 5 | 635 | |
| | | | 25 | 7 | 635 | |
| | | | 30 | 10 | 620 | |
| | | | 35 | 13 | 610 | |
| | | | 40 | 15 | 615 | |
| | | | 50 | 24 | 590 | |
| | | | 55 | 30 | 570 | |
| | | | 60 | 36 | 550 | |
| 3 | m-nitro- | 80.2 | - | - | 640 | Homogenous |
| | cinnamoyl- | (0.2) | 5 | 0 | 640 | dense |
| | ferrocene | | 10 | 2 | 640 | varnished |
| | 0.00143 | | 15 | 2 | 640 | deposit |
| | (0.000229) | | 20 | 3 | 635 | |
| | | | 25 | 3 | 635 | |
| | | | 30 | 5 | 630 | |
| | | | 35 | 6 | 630 | |
| | | | 40 | 8 | 625 | |
| | | | 45 | 9 | 610 | |
| | | | 50 | 10 | 600 | |
| | | | 60 | 10 | 600 | |
| 4 | o-chloro- | 81.8 | - | - | 640 | Homogeneous |
| | cinnamoyl- | (1.8) | 5 | 4 | 640 | dense |
| | ferrocene | | 10 | 8 | 630 | varnished |
| | 0.0287 | | 15 | 12 | 620 | deposit |
| | (0.00455) | | 20 | 17 | 600 | |
| | | | 25 | 27 | 590 | |
| | | | 30 | 32 | 580 | |
| | | | 35 | 40 | 570 | |
| | | | 40 | 55 | 550 | |
| | | | 45 | 58 | 490 | |
| | | | 50 | stop | | |
| 5 | o-chloro- | 81.7 | - | - | 640 | Homogeneous |
| | cinnamoyl- | (0.9) | 5 | 0 | 640 | dense |
| | ferrocene | | 10 | 1 | 640 | varnished |
| | 0.0144 | | 15 | 2 | 640 | deposit |
| | (0.00229) | | 20 | 4 | 635 | |
| | | | 25 | 7 | 635 | |
| | | | 30 | 9 | 630 | |
| | | | 35 | 14 | 620 | |
| | | | 40 | 16 | 600 | |
| | | | 45 | 21 | 590 | |
| | | | 50 | 28 | 570 | |
| | | | 60 | 38 | 540 | |
| 6 | o-chloro- | 80.2 | - | - | 640 | Homogeneous |
| | cinnamoyl- | (0.2) | 5 | 0 | 640 | dense |
| | ferrocene | | 10 | 2 | 640 | varnished |
| | 0.00144 | | 15 | 3 | 635 | deposit |
| | (0.000229) | | 20 | 4 | 630 | |
| | | | 25 | 4 | 630 | |
| | | | 30 | 5 | 620 | |
| | | | 35 | 6 | 610 | |
| | | | 40 | 8 | 610 | |
| | | | 45 | 9 | 600 | |
| | | | 50 | 10 | 600 | |
| | | | 55 | 10 | 600 | |
| | | | 60 | 10 | 600 | |
| 7 | α-hydroxy- | 82.0 | - | - | 640 | Crumbly microporous deposit |
| | isopropyl | (2.0) | 5 | 12 | 610 | |
| | ferrocene | | 10 | 22 | 530 | |
| | 0.02 | | 15 | 34 | 500 | |
| | (0.00458) | | 20 | 40 | 450 | |
| | | | 25 | 55 | 400 | |
| | | | 30 | 52 | 410 | |
| | | | 35 | 52 | 415 | |
| | | | 40 | 55 | 400 | |
| | | | 45 | 50 | 410 | |
| | | | 50 | 50 | 415 | |
| | | | 55 | 54 | 400 | |
| | | | 60 | 51 | 410 | |
| 8 | α-hydroxy- | 82.5 | - | - | 640 | Crumbly microporous deposit |
| | isopropyl- | (2.5) | 5 | 22 | 530 | |
| | ferrocene | | 10 | 37 | 500 | |
| | 0.025 | | 15 | 59 | 320 | |
| | (0.00572) | | 20 | 68 | 320 | |
| | | | 25 | 68 | 320 | |
| | | | 30 | 72 | 310 | |
| | | | 35 | stop | | |
| 9 | α-hydroxy- | 81.1 | - | - | 640 | Crumbly |
| | isopropyl | (1.8) | 5 | 3 | 630 | microporous |
| | ferrocene | | 10 | 7 | 620 | deposit |
| | 0.01 | | 15 | 11 | 590 | |
| | (0.00229) | | 20 | 15 | 580 | |
| | | | 25 | 20 | 570 | |
| | | | 30 | 24 | 560 | |
| | | | 35 | 27 | 545 | |
| | | | 40 | 31 | 530 | |
| | | | 45 | 34 | 510 | |
| | | | 50 | 31 | 520 | |
| | | | 55 | 32 | 520 | |
| | | | 60 | 30 | 510 | |
| 10 | α-hydroxy- | 80.3 | - | - | 640 | Crumbly |
| | isopropyl | (0.3) | 5 | 2 | 640 | microporous |
| | ferrocene | | 10 | 2 | 640 | deposit |
| | 0.001 | | 15 | 3 | 640 | |
| | (0.000229) | | 20 | 4 | 640 | |
| | | | 25 | 5 | 630 | |
| | | | 30 | 6 | 630 | |
| | | | 35 | 6 | 620 | |
| | | | 40 | 8 | 620 | |
| | | | 45 | 9 | 600 | |
| | | | 50 | 10 | 600 | |
| | | | 60 | 9 | 600 | |

| | | | | | | |
|---|---|---|---|---|---|---|
| Notes: 1. Example No. | | | | | | |
| 2. Additive, dosage percent (content of additive based on the weight percent content of Fe). | | | | | | |
| 3. Fuel composition octane number by an engine method (increased octane number). | | | | | | |
| 4. Time in hours. | | | | | | |
| 5. Increased weight of the spark plug, mg. | | | | | | |
| 6. Sparking gap of the plug, µm. | | | | | | |
| 7. Iron oxide deposit on the plug electrodes (magnification X50). | | | | | | |

The data in the Table show that the iron oxide deposits formed on combustion of the fuel composition according to the invention and on combustion of the prior art fuel compositions have different natures, and that their accumulation on the sparking plug proceeds at different rates. Thus, the known prior art fuel produces dense solid varnished iron oxide deposits. However, on combustion of the fuel composition according to the present invention crumbly microporous deposits are formed.

Thus, Examples 7 to 10 (fuel composition according to the invention) indicate that the accumulation of iron oxide deposits up to the equal weight state (50 to 55 mg) proceeds for 25 hours and remains at this level for a long period of the tests. At the same time the known prior art fuel composition containing an equivalent amount of iron (458 x 10⁻⁵ percent by weight) in the fuel mixture when the similar amount of iron oxide deposit (50 to 55 mg) for a more extended period of time (35 to 40 hours) leads to a stoppage of the engine (see Examples 1,4).

However, the step of decreasing the content of the anti-knock ferrocene additives by iron to 229 x 10⁻⁵ percent by weight as for the fuel composition according to the invention increases the time to achieve the equal weight state of iron oxide deposit up to a level of 40 hours and to diminish the deposit value in the equal weight state down to 30 to 34 mg (see Example 9).

At the same time, in the case of the known prior art fuel composition a similar amount of iron oxide deposit (30 to 34 mg) accumulates for 50 to 55 hours and for the next 5 to 10 hours a further increase of the iron oxide deposit occurs up to 35 to 38 mg. This feature shows that in the operation of the engine the iron oxide deposits will accumulate permanently.

Thus, the use of α-hydroxyisopropyl ferrocene as an anti-knock additive serves to increase the life of sparking plugs without worsening the performances of the engine.

In addition, the use of α-hydroxyisopropyl ferrocene in the fuel composition increases by 15 to 20 percent the growth of octane number as compared to m-nitrocinnamoylferrocene and o-chlorocinnamoyl ferrocene at the equivalent content of iron.

The use of α-hydroxyisopropyl ferrocene increases by two times the content of iron as compared to the prior art fuel compositions containing m-nitrocinnamoylferrocene without inflicting any damage to the operation of sparking plug of the engine, increasing the octane number by 1.1 to 1.2 units (see Example 8).

In addition the use of α-hydroxyisopropyl ferrocene reduces the toxicity rate of combustion products.

The lower limit of the use of α-hydroxyisopropyl ferrocene is 0.001 percent (see Example 10),the upper limit is 0.02 percent (see Example 8) and corresponds to the maximum possible content at which a faultless operation of the engine is provided.

## Claims

1. A hydrocarbon based fuel composition suitable for spark ignition internal combustion engines, which comprises 0.001 %0.02% by weight of

2. A composition according to claim 1 wherein the fuel comprises
54-56% by weight of aromatic hydrocarbons,
12-13% by weight of normal alkanes,
29-31% by weight of isoalkanes and
1-2% by weight of naphthenes.

3. A composition according to claim 1 or 2 wherein the fuel has an octane number of 80.

4. Use of as an anti-knock additive suitable for fuels.

## Patentansprüche

1. Auf Kohlenwasserstoff basierende Kraftstoff-Zusammensetzung, geeignet für . Verbrennungsmotoren mit Funkenzündung, welche umfaßt:
0,001 - 0,02 Gewichts-% von

2. Zusammensetzung nach Anspruch 1, bei der der Kraftstoff umfaßt:
54-56 Gew.-% aromatische Kohlenwasserstoffe,
12-13 Gew.-% normale Alkane,
29-31 Gew.-% Isoalkane und
1-2 Gew.-% Naphthene.

3. Zusammensetzung nach Anspruch 1 oder 2, bei der der Kraftstoff eine Oktanzahl von 80 aufweist.

4. Verwendung von als einem für Kraftstoffe geeigneten Antiklopfmittel.

## Revendications

1. Composition de carburant à base d'hydrocarbures, qui convient pour des moteurs à combustion interne et allumage par étincelle et qui contient de 0,001 % à 0,02 % en poids de

2. Composition conforme à la revendication 1, dans laquelle le carburant contient :
- de 54 à 56 % en poids d'hydrocarbures aromatiques,
- de 12 à 13 % en poids d'alcanes normaux,
- de 29 à 31 % en poids d'isoalcanes, et
- de 1 à 2 % en poids de naphtènes.

3. Composition conforme à la revendication 1 ou 2. dans laquelle le carburant présente un indice d'octane de 80.

4. Emploi de comme adjuvant antidétonant approprié pour carburants.
